

Feb. 10, 1942.

E. A. ANDERSON ET AL

2,272,390

ALLOY

Filed Jan. 16, 1940

3 Sheets-Sheet 1



TENSILE STRENGTH.

Trilinear chart of certain Zn-Mn-Cu alloys containing 0.15% Al. Tensile strengths in pounds per sq. in. shown by contours. Alloys cold chamber die-cast from mixtures of commercial grades of metals and contain various impurities, particularly Fe, in proportions ranging from .1% to .7%.

INVENTORS  
Edmund A. Anderson  
Gerald Edmunds  
BY

Dennis Davis, Rogers and Hammond  
ATTORNEYS

Feb. 10, 1942.

E. A. ANDERSON ET AL

2,272,390

ALLOY

Filed Jan. 16, 1940

3 Sheets-Sheet 2



IMPACT STRENGTH.

Trilinear chart of Zn-Mn-Cu alloys  
(of Fig. 1) containing 0.15% Al. and  
having tensile strengths of about 60,000  
lbs. per sq. in. or more. Impact strengths  
in foot pounds for bars  $\frac{1}{4}$ " sq. shown by  
solid contour lines.

INVENTORS  
Edmund A. Anderson  
Gerald Edmunds

BY  
Pennie, Davis, Newman and Lamonds

ATTORNEYS

Feb. 10, 1942.

E. A. ANDERSON ET AL

2,272,390

ALLOY

Filed Jan. 16, 1940

3 Sheets-Sheet 3



Trilinear chart of Zn-Mn-Cu alloys  
(of Fig. 1), containing 0.15% Al. Brinell  
hardness numbers of certain of these  
alloys plotted.

INVENTORS  
Edmund A. Anderson  
Gerald Edmunds  
BY

Connie, Davis, Marvin and Edmunds  
ATTORNEYS

## UNITED STATES PATENT OFFICE

2,272,390

## ALLOY

Edmund A. Anderson and Gerald Edmunds, Palmerston, Pa., assignors to The New Jersey Zinc Company, New York, N. Y., a corporation of New Jersey

Application January 16, 1940, Serial No. 314,086

9 Claims. (Cl. 75—178)

This invention relates to zinc base alloys and provides new alloys containing zinc, manganese, and aluminum (and, preferably, also copper) having superior mechanical properties. The alloys of our invention have an appearance similar to that of white metal alloys.

As a result of our investigations, we have discovered new zinc alloys containing certain proportions of manganese, and aluminum (and preferably also copper) which, as cast, have an impact strength of about one foot-pound per one-quarter square inch cross section or more, a tensile strength of about 60,000 pounds per square inch or higher, and high creep resistance. They may be formed into intricate shapes of accurate configuration by die casting, and are also amenable to casting by other methods.

All percentages given hereinafter are percentages by weight, and on this basis the alloys of our invention contain aluminum in proportions ranging from 0.02% to about 5% (but preferably from 0.1 to 2%), together with manganese in the proportions ranging from about 7.5% to about 48.5%, and (preferably) copper in proportions not exceeding about 26½%, the balance of the alloy being principally zinc, except that the alloys may contain a substantial percentage of iron. The proportion of iron which may be present is dependent upon the copper and manganese contents, but in general the alloys should not contain more than about 6% of iron.

In the manufacture of the alloys of our invention, it is not essential in all cases to employ high grade manganese, for the impurities that may occur in the ordinary commercial grades of manganese may be included in our alloys in some cases without too serious effect upon the properties thereof. Manganese suitable for use in the practice of our invention may contain minor proportions of silicon, phosphorus, carbon, nitrogen, and other impurities. We prefer, however, to use manganese of high purity, since impurities in the manganese may degrade the mechanical properties of the alloy and, in particular, cause the presence of hard particles that may interfere with machining and buffing.

The alloys of our invention, their composition, and their mechanical properties, particularly in cold chamber die-cast form, are described more fully hereinafter with reference to the accompanying drawings, Figs. 1, 2, and 3, which are trilinear charts representing the zinc corner of the Zn-Cu-Mn system, extending to 30% Cu and 50% Mn and in which:

Fig. 1 shows the approximate proportions of zinc, copper and manganese to be employed (together with certain proportions of aluminum) in the manufacture of alloys of our invention having impact strengths of about 1 foot-pound or more per one-quarter inch square cross section, (in the specification and claims the term "impact strength" refers to values obtained in a Charpy impact test on unnotched test bars), and tensile strengths of about 60,000 pounds per square inch or better;

Fig. 2 shows the impact strength of the alloys by means of contour lines; and

Fig. 3 shows the Brinell hardness numbers of certain alloys of our invention.

In Fig. 1, the contour line A' demarcates the range of composition in which the alloys have a tensile strength of 60,000 pounds per square inch or better. The contour line B' demarcates the range of composition in which the alloys have a tensile strength of 70,000 pounds per square inch or better. The contour line C' encloses the range of composition in which the alloys have a tensile strength of 80,000 pounds per square inch or better. The contour line D' encloses the area in which the alloys have a tensile strength of 90,000 pounds per square inch or better. The dotted line E', E'', E''' is the same as the line E', E'', E''' in Fig. 2, and encloses the range of composition in which the alloys have an impact strength of 1 foot-pound or more per one-quarter inch square cross section. The curved portion E' of this line is a contour line; the straight portions E'' and E''' represent boundaries on the zinc-poor side of which difficulties are encountered in the preparation and casting of the alloys. It will be noted that the contour lines A' and B' do

not enclose an area, being open towards the manganese corner of the diagram. The line E'''<sup>10</sup>, however, closes the areas delimited by contour lines A' and B'. Thus, the area delimited by A' and E'''<sup>15</sup> contains useful alloy compositions having a tensile strength of 60,000 pounds per square inch or better, and the area delimited by B' and E'''<sup>20</sup> contains useful alloy compositions having a tensile strength of 70,000 pounds per square inch or better.

In Fig. 2, the contour line E' indicates the range of composition of alloys having an impact strength of 1 foot-pound or more per one-quarter inch square cross section. As has been explained in the discussion of Fig. 1, the straight dotted lines E'' and E'''<sup>15</sup> show limits beyond which towards the zinc-poor field of alloy compositions difficulties are encountered in the preparation and casting of the alloys. Contour line F' indicates the range of composition of alloys having an impact strength of 2 foot-pounds or more per one-quarter inch square cross section. Contour line G' indicates the range of composition of alloys having an impact strength of 4 foot-pounds or more per one-quarter inch square cross section. The areas enclosed by contour lines F' and G' are closed by the straight boundary E'''<sup>25</sup>. Contour line H' encloses the range of composition in which the alloys have an impact strength of 8 foot-pounds or more per one-quarter inch square cross section.

For convenience of reference, contour line A' and a portion of the boundary line E'''<sup>30</sup> are inserted in Fig. 3.

As shown in the trilinear charts, the proportions of copper and manganese are interdependent in their effect upon the tensile strength and other properties of the alloys. The following tables give the approximate manganese range for specific copper contents (Table I) and the approximate copper range for specific manganese contents (Table II). As shown in Fig. 1, the contour A' (drawn through points representing the composition of alloys having tensile strength of about 60,000 pounds) and the contour line E' (drawn through points representing the composition of alloys having impact strength of about 1 foot-pound per one-quarter inch square bar)<sup>40</sup> are roughly coincident and define approximately the same area. In short, the alloys of our invention have tensile strengths of about 60,000 pounds per square inch or more, together with impact strengths of about 1 foot-pound plus. The values in Tables I and II represent points on both contours A' and E', depending upon which is outermost on the chart. Thus, in order to obtain alloys that may be cast readily and that have, as cast, tensile strength of approximately 60,000 pounds per square inch or more and impact strength of about 1 foot-pound per one-quarter inch square section or more, the approximate manganese ranges for given copper contents are as follows:

TABLE I

| Points on Fig. 1 | Per cent Cu | Per cent Mn       |
|------------------|-------------|-------------------|
| 10-10''          | 0           | 33-48             |
| 11-11'           | 5           | 26-47             |
| 12-12'           | 10          | 18-45             |
| 13-13'           | 15          | 12-41             |
| 14-14'           | 20          | 7+36              |
| 15-15', 15''     | 25          | 17-26 and also 31 |
| 16-16'           | 26          | 18-23             |

To express the relationship of copper and manganese contents in another way, the approximate limits of copper content for given manganese contents are as follows:

5

TABLE II

10

| Per cent Mn | Per cent Cu |
|-------------|-------------|
| 48          | 0-2         |
| 45          | 0-9         |
| 40          | 0-16        |
| 35          | 0-21        |
| 30          | 2-24        |
| 25          | 6-25        |
| 20          | 8-27        |
| 15          | 12-22       |
| 10          | 16-20       |

As shown in Fig. 1 (area A) an alloy of our invention containing 0.15% aluminum, 38.5% manganese, and substantially no copper, the balance being substantially all zinc, has a tensile strength as cast of about 60,000 pounds per square inch (points 10'-10''). The same tensile strength is found in alloys with the same aluminum content but with various proportions of manganese and copper as follows:

Area "A," Boundary "A"

| Point on Fig. 1 | Approximate analyses of alloys having tensile strength of about 60,000 pounds per square inch |             |             |
|-----------------|-----------------------------------------------------------------------------------------------|-------------|-------------|
|                 | Per cent Al                                                                                   | Per cent Cu | Per cent Mn |
| 17              | 0.15                                                                                          | 6           | 25          |
| 18              | 0.15                                                                                          | 11.3        | 16          |
| 19              | 0.15                                                                                          | 18          | 8.8         |
| 20              | 0.15                                                                                          | 20          | 12.7        |
| 16              | 0.15                                                                                          | 26          | 17.5        |
| 21              | 0.15                                                                                          | 26.4        | 20          |
| 22              | 0.15                                                                                          | 23.3        | 30          |
| 23              | 0.15                                                                                          | 7.5         | 45.7        |

55 Still higher tensile strengths are obtainable by differently proportioning the manganese and copper contents of the alloys of our invention.

Certain of the alloys of our invention have, as cast, tensile strengths of about 70,000 pounds per square inch or higher. These alloys contain in addition to about 0.02% to about 2% aluminum, from about 1.5% to about 24% copper, and about 11% to about 48.5% manganese, the balance of the alloy (except for a relatively small iron content) consisting essentially of zinc. In these alloys the copper and manganese contents are so related as to define points lying substantially in the area B on the trilinear chart (Fig. 1).

Some of the alloys have, as cast, a tensile strength of 80,000 pounds per square inch or more and contain in addition to aluminum ranging from about 0.02% to about 2%, copper in proportions ranging from about 9% to about 22.5%, and manganese ranging in proportions from about 13.5% to about 34.5%, the balance of

78

the alloy as in the previous cases consisting essentially of zinc, with or without a relatively small proportion of iron, and the copper and manganese contents of the alloys being such as to define a point lying substantially in the area C on the trilinear chart (Fig. 1).

To obtain alloys having a tensile strength of about 90,000 pounds per square inch or more, in accordance with our invention the aluminum content of the alloys should range from about 0.02% to about 2% and should be accompanied by manganese, in proportions ranging from about 15% to about 22½%, and copper in proportions ranging from about 15% to about 22%. These alloys have manganese and copper contents so related as to define points lying substantially in the area D of the trilinear chart (Fig. 1).

In short, those alloys having a tensile strength of 70,000 pounds per square inch or more, are of analyses that fall within the area B on Fig. 1; those having a tensile strength of at least 80,000 pounds per square inch are those having copper and manganese contents that fall within the area C on Fig. 1, while those of tensile strengths of 90,000 pounds or more per square inch are those having manganese and copper contents enclosed within the area D on Fig. 1. For example, those alloys containing 0.15% aluminum, 20% copper and 16% to 22.5% manganese, the balance being substantially all zinc, have tensile strengths of at least 90,000 pounds per square inch.

It will be observed that the range of useful alloys having impact strengths of 1 foot-pound or more per one-quarter inch square section is defined by the area E, enclosed by the impact strength contour line E' on the trilinear charts running from point 10 (0% Cu, 33.3% Mn) through point 24 (16% Cu, 10% Mn), point 14 (20% Cu, 7.5% Mn), point 25 (20.2% Cu, 10% Mn), point 26 (23% Cu, 20% Mn), point 27 (22% Cu, 25.5% Mn) to point 15' (25% Cu, 31% Mn); the straight line E'' running from point 15' to point 28 (11% Cu, 44.5% Mn); and the straight line E''' running from point 28 to point 10'' (0% Cu, 48.5% Mn). The line E''' in addition to establishing part of the boundary of area E, marks the limit of areas A and B on Fig. 1, and areas F and G on Fig. 2.

The straight lines E'' and E''' are not contour lines, but, in the case of compositions lying substantially above or outside these lines, i. e., on the zinc-poor side of these lines, difficulties are encountered in the preparation and handling of the alloys.

All of the alloys of our invention have, as shown in Fig. 2, adequately high impact strength, that is to say, they are not brittle. The area F enclosed by the contour line F' on Fig. 2 indicates the proportions of copper and manganese employed in alloys of our invention, together with aluminum (the balance of the alloy being substantially all zinc) to obtain impact strengths of at least 2 foot-pounds in a cold chamber die-cast bar with a one-quarter inch square section. Still higher impact strengths (i. e., 4 foot-pounds per quarter inch square section, or better) are obtained with compositions falling within the area G bounded by the contour line G' on Fig. 2, and impact strengths of 8 foot-pounds per one-quarter inch square, or better, are obtained with alloys of compositions falling within the area H bounded by the contour line H' on Fig. 2.

Approximate limits of the several areas in

terms of the copper and manganese contents they represent are as follows:

| 5       | Tensile strength, pounds per sq. in. | Area | Copper range | Manganese range |
|---------|--------------------------------------|------|--------------|-----------------|
| 60,000+ |                                      | A    | 0 - 26½      | 8½ - 48½        |
| 70,000+ |                                      | B    | 1½ - 24      | 11 - 48         |
| 80,000+ |                                      | C    | 9 - 22½      | 13½ - 34½       |
| 90,000+ |                                      | D    | 15 - 22      | 15 - 22½        |

| 15 | Impact strength foot-pounds per ¼ in. square | Area | Copper range | Manganese range |
|----|----------------------------------------------|------|--------------|-----------------|
| 1+ |                                              | E    | 0 - 25       | 7½ - 48½        |
| 2+ |                                              | F    | 0 - 23       | 12 - 48½        |
| 4+ |                                              | G    | 0 - 21½      | 16½ - 48½       |
| 8+ |                                              | H    | 7½ - 20      | 20 - 38         |

As indicated by Fig. 3, the alloys of our invention are relatively hard, having a Brinell hardness ranging from 262 to 140. It will be observed that in general the alloys having a relatively high copper content are hardest, while those with a relatively low copper content are in general relatively soft.

Alloys of our invention are not subject to the temperature embrittlement encountered in many zinc alloys at very low temperatures. Thus, an alloy of our invention containing 24% to 25% manganese, 15.2% to 15.5% copper, 0.15% to 0.18% aluminum (the remainder being special high-grade zinc of high purity) was tested for impact strength and tensile strength at low temperatures and was found not to become brittle, even at temperatures as low as -40° C.

Alloys of our invention have high creep resistance. Alloys containing 24-25% manganese, 15.2-15.5% copper, and 0.15-0.18% aluminum, the remainder being special high-grade zinc, were tested for creep resistance at 25° C. under bending stresses equivalent to maximum fiber stresses in tension up to 70,000 pounds per square inch. No creep was detected during three days. In contrast, heretofore customary zinc base die-casting alloys suffered detectable creep in three days under a stress of 2,500 pounds per square inch, other conditions being the same.

The modulus of elasticity of alloys of our invention as indicated by beam deflections observed during the above reported creep tests was found to be about 14,000,000 pounds per square inch, which is greater than that of any zinc base die-casting alloys known to us.

Moreover, the alloys of our invention possess apparent rigidity or stiffness to a degree greater than that of any other zinc alloys of reasonable ductility.

All of the alloys of our invention are machinable.

The alloys of our invention manifest good resistance to atmospheric corrosion. Further, water immersion tests of alloys containing 25% Mn, 15% Cu and 0.15% Al (the balance being substantially all zinc) showed a corrosion resistance roughly comparable to that of the zinc base die-casting alloys Nos. XXI, XXIII, and XXV of A. S. T. M. tentative specifications E86-38T, 1938.

The preferred group of alloys of our invention consists of those within the range of compositions delineated by the 8 foot-pound con-

tour (H') on the impact strength chart (Fig. 2, area H). These alloys all have (as cast) tensile strengths ranging from about 75,000 to 97,000 pounds per square inch and tensile elongation values from about 1% to 6% in a two inch gage length. By way of example, the following alloys within the preferred range are cited.

|                                                                | Alloy  |        |        |        |        |
|----------------------------------------------------------------|--------|--------|--------|--------|--------|
|                                                                | I      | II     | III    | IV     | V      |
| Analyzed percent Mn.....                                       | 22.2   | 24.7   | 29.6   | 34.2   | 21.6   |
| Analyzed percent Cu.....                                       | 17.5   | 15.4   | 14.4   | 10.0   | 18.3   |
| Analyzed percent Al.....                                       | 0.15   | 0.17   | 0.18   | 0.18   | 0.14   |
| Analyzed percent Fe.....                                       | 0.17   | 0.19   | 0.23   | 0.28   | 0.18   |
| Tensile strength, lbs. per square in.....                      | 90,200 | 89,100 | 84,900 | 81,200 | 97,300 |
| Tensile elongation, percent in 2 in.....                       | 2      | 6      | 2      | 2      | 3      |
| Impact strength, foot-pounds on $\frac{1}{4}$ in. sq. bar..... | 12.9   | 18     | 12.1   | 11.9   | 12.7   |
| Brinell hardness number.....                                   | 167    | 158    | 161    | 159    | 184    |

It will be observed that the alloys lying within the preferred range possess, as cast, remarkably superior characteristics which favor their use in the manufacture of a great variety of articles by inexpensive processes, such as die casting.

As indicated hereinbefore, aluminum is an essential ingredient in the alloys of our invention. The presence of the aluminum not only improves the casting characteristics of the alloys, but also tends to suppress oxidation of the surfaces of the hot casting. The presence of the aluminum in the alloys of our invention enables castings made thereof to be cooled in air without serious discoloration. An unsightly brown film forms on the surface of air-cooled castings of similar Zn-Cu-Mn alloys without the aluminum. Moreover, the presence of the aluminum in the alloy within the range specified, i. e., 0.02% to about 5%, reduces dross formation on the molten alloy during casting operations and tends to impart an attractive silvery appearance to the resulting casting. When aluminum is not present, a tenacious brown film tends to form on the molten alloy, interfering with pouring and making difficult the production of a casting having a smooth surface. However, an aluminum content of more than about 5% cannot be tolerated because of the deleterious effect thereof upon the mechanical properties of the alloys. In case the aluminum content exceeds 2%, the tolerance for impurities is limited. The effect of aluminum upon relatively impure alloys is illustrated in the following table:

|                                                                | Alloy  |        |        |        |
|----------------------------------------------------------------|--------|--------|--------|--------|
|                                                                | VI     | VII    | VIII   | IX     |
| Analyzed percent of Mn.....                                    | 24.7   | 24.7   | 23.8   | 21.5   |
| Analyzed percent of Cu.....                                    | 15.4   | 15.4   | 15.4   | 13.3   |
| Analyzed percent of Al.....                                    | 0.023  | 0.45   | 1.2    | 5.3    |
| Analyzed percent of Fe.....                                    | 0.19   | 0.21   | 0.19   | 0.21   |
| Tensile strength, lbs. per square inch.....                    | 90,600 | 86,100 | 89,200 | 28,700 |
| Tensile elongation, percent in 2 in.....                       | 5      | 2      | 1      | -----  |
| Impact strength, foot-pounds on $\frac{1}{4}$ in. sq. bar..... | 16     | 11     | 3.1    | 0.4    |
| Brinell hardness number.....                                   | 166    | 172    | 191    | 214    |

The inclusion of up to 6% iron in the alloys of our invention is permissible. The tolerance for iron of the particular alloy depends upon its copper and manganese and impurity contents and is greater for some compositions. The ef-

fect of the inclusion of iron upon relatively impure alloys is shown by the following data:

|                                                                | 5      | Alloy  |        |        |      |
|----------------------------------------------------------------|--------|--------|--------|--------|------|
|                                                                |        | X      | XI     | XII    | XIII |
| Analyzed percent Mn.....                                       | 24.4   | 23.5   | 21.0   | 24.0   |      |
| Analyzed percent Cu.....                                       | 15.5   | 14.4   | 13.5   | 16.4   |      |
| Analyzed percent Al.....                                       | 0.18   | 0.090  | 0.085  |        |      |
| Analyzed percent Fe.....                                       | 0.19   | 2.2    | 4.9    | 5.4    |      |
| Tensile strength, lbs. per square inch.....                    | 88,500 | 83,000 | 87,900 | 77,500 |      |
| Tensile elongation, percent in 2 in.....                       | 4      | 2      | 1      | 0      |      |
| Impact strength, foot-pounds on $\frac{1}{4}$ in. sq. bar..... | 18     | 11     | 4.7    | 3.8    |      |
| Brinell hardness number.....                                   | 156    | 158    | 158    | 178    |      |

\*Not analyzed, synthetic composition, 0.15% Al.

All of the specific alloys described herein were made from zinc having a purity of at least 99.98%.

The alloys of our invention can be prepared with the ingredients charged into the crucible in the form of unalloyed metals or alloys of these with each other. We prefer to melt the alloys in a crucible substantially non-reactive to the alloys. We have found clay-silicon carbide and cast iron crucibles to be satisfactory. It is helpful in many cases to protect the surface of the molten alloy with a nonreactive gas, e. g., hydrogen.

As indicated hereinbefore, all of the alloys of our invention can be die cast and offer certain advantages over heretofore customary zinc alloys that can be die cast because of their greater strength and hardness. However, certain alloys of our invention have been gravity cast in permanent metal moulds and also gravity cast in sand moulds. Although some differences in properties of the alloys of our invention are induced by the method of casting, the alloys of our invention in general exhibit superior properties as compared with heretofore customary zinc alloys, irrespective of the particular method of casting.

We claim:

1. An alloy having as cast an impact strength of at least about 1 foot-pound per  $\frac{1}{4}$  inch square section and containing about 0.02 per cent to about 5 per cent aluminum, copper in effective amount up to about 26 per cent and about 7.5 per cent to about 48.5 per cent manganese, the balance of the alloy being substantially all zinc and the copper and the manganese contents of the alloy being so related to each other as to define a point on the accompanying trilinear chart (Fig. 2) lying within the area E defined by the line connecting the following series of points:

| 60  | Point No. | Per cent Cu | Per cent Mn |
|-----|-----------|-------------|-------------|
| 10  |           | 0           | 33.3        |
| 24  |           | 16          | 10          |
| 14  |           | 20          | 7.5         |
| 25  |           | 20.2        | 10          |
| 26  |           | 23          | 20          |
| 27  |           | 22          | 25.5        |
| 15" |           | 25          | 31          |
| 28  |           | 11          | 44.5        |
| 10" |           | 0           | 48.5        |
| 10  |           | 0           | 33.3        |

2. An alloy having as cast an impact strength of at least about 2 foot-pounds per  $\frac{1}{4}$  inch square section and containing about 0.02 per cent to about 2 per cent aluminum, copper in effective amount up to about 23 per cent, and manganese in proportions ranging from about 12 per cent to

about 48½ per cent, substantially all of the balance of the alloy being zinc, the copper and manganese in the alloy being so related to each other as to define a point on the accompanying trilinear chart (Fig. 2) lying within the area F defined by the line connecting the following series of points:

| Per cent Cu | Per cent Mn |
|-------------|-------------|
| 0           | 38          |
| 4.5         | 30          |
| 12.5        | 17.5        |
| 17.5        | 12          |
| 22.5        | 17.5        |
| 23          | 20          |
| 20          | 30          |
| 17          | 35          |
| 14          | 40          |
| 9           | 45          |
| 0           | 48.5        |
| 0           | 38          |

3. An alloy having as cast an impact strength of at least about 4 foot-pounds per ¼ inch square section and containing about 0.02 per cent to about 2 per cent aluminum, copper in effective amount up to about 21½ per cent, and about 16½ per cent to about 48½ per cent manganese, substantially all of the balance of the alloy being zinc, the copper and manganese contents of the alloy being such as to define a point on the accompanying trilinear chart (Fig. 2) lying within the area G defined by the line connecting the following series of points:

| Per cent Cu | Per cent Mn |
|-------------|-------------|
| 0           | 43          |
| 2.5         | 40          |
| 4.5         | 35          |
| 6.5         | 30          |
| 8.5         | 25          |
| 12.5        | 20          |
| 15          | 17.5        |
| 17.5        | 16.5        |
| 20          | 16.8        |
| 21.5        | 20          |
| 20          | 25          |
| 15          | 35          |
| 12          | 40          |
| 4           | 47          |
| 0           | 48.5        |
| 0           | 43          |

4. An alloy having as cast an impact strength of at least about 8 foot-pounds per ¼ inch square section and containing about 0.02 per cent to about 2 per cent aluminum, about 7½ per cent to about 20 per cent copper, and about 20 per cent to about 38 per cent manganese, substantially all of the balance of the alloy being zinc, and the copper and manganese contents of the alloy being so related as to define a point on the accompanying trilinear chart (Fig. 2) lying within the area H defined by the line connecting the following series of points:

| Percent Cu | Percent Mn |
|------------|------------|
| 7.5        | 37         |
| 15         | 22         |
| 18.5       | 20         |
| 20         | 21.5       |
| 18.5       | 25         |
| 16         | 30         |
| 13         | 35         |
| 10         | 37.5       |
| 8.5        | 38         |
| 7.5        | 37         |

5. An alloy having as cast a tensile strength of at least about 60,000 pounds per square inch and containing about 0.02 per cent to about 5

per cent aluminum, copper in effective amount up to about 26½ per cent and about 8½ per cent to about 48½ per cent manganese, substantially all of the balance of the alloy being zinc and the copper and manganese contents of the alloy being such as to define a point on the accompanying trilinear chart (Fig. 1) lying within the area A defined by the line connecting the following series of points:

| Point No. | Percent Cu | Percent Mn |
|-----------|------------|------------|
| 10'       | 0          | 38         |
| 17        | 6          | 25         |
| 15        | 11.3       | 16         |
| 18        | 18         | 8.5        |
| 19        | 20         | 12.7       |
| 20        | 25         | 17.5       |
| 16        | 26.5       | 20         |
| 21        | 23.3       | 30         |
| 22        | 7.5        | 45.7       |
| 23        | 0          | 48.5       |
| 10''      | 0          | 38         |
| 20        | 10'        |            |

6. An alloy having as cast a tensile strength of at least about 70,000 pounds per square inch and containing about 0.02 per cent to about 2 per cent aluminum, about 1.5 per cent to about 24.5 per cent copper and about 11 per cent to about 48 per cent manganese, substantially all of the balance of the alloy being zinc, the copper and manganese contents of the alloy being so related as to define a point on the accompanying trilinear chart (Fig. 1) lying within the area B defined by the line connecting the following series of points:

| Percent Cu | Percent Mn |
|------------|------------|
| 1.5        | 48         |
| 5          | 37.5       |
| 7.5        | 27.5       |
| 8.5        | 23.5       |
| 12.5       | 16.5       |
| 18         | 11         |
| 24         | 17.5       |
| 24.5       | 20         |
| 23         | 27.5       |
| 22.5       | 29.5       |
| 18.5       | 33         |
| 6          | 46.5       |
| 1.5        | 48         |

7. An alloy having as cast a tensile strength of at least about 80,000 pounds per square inch and containing about 0.02 per cent to about 2 per cent aluminum, about 9 per cent to about 22½ per cent copper and about 13½ per cent to about 34½ per cent manganese, substantially all of the balance of the alloy being zinc and the copper and manganese contents of the alloy being such as to define a point on the accompanying trilinear chart (Fig. 1) lying within the area C defined by the line connecting the following series of points:

| Percent Cu | Percent Mn |
|------------|------------|
| 10         | 34.5       |
| 9          | 26         |
| 13         | 17.5       |
| 18         | 13.5       |
| 22.5       | 18         |
| 21.5       | 29         |
| 18         | 34         |
| 10         | 34.5       |

8. An alloy having as cast a tensile strength of at least about 90,000 pounds per square inch and containing about 0.02 per cent to about 2 per cent aluminum, about 15 per cent to about

22 per cent copper and about 15 per cent to about 22½ per cent manganese, substantially all of the balance of the alloy being zinc, and the copper and manganese contents of the alloy being such as to define a point lying within the area D on the accompanying trilinear chart (Fig. 1) delineated by the line D' passing through the following series of points:

| Per cent Cu | Per cent Mn |
|-------------|-------------|
| 20          | 22.5        |
| 17.5        | 22          |
| 15.5        | 20          |
| 15          | 18.5        |
| 15.5        | 17.5        |
| 17.5        | 15.5        |
| 18          | 15          |
| 22          | 17.5        |
| 22          | 20          |
| 21.5        | 21.5        |
| 20          | 22.5        |

9. An alloy containing about 0.02 per cent to about 5 per cent aluminum and about 7.5 per cent to about 48.5 per cent manganese, substantially all of the balance of the alloy being elements selected from the group consisting of zinc and copper, the copper being present in effective amount up to about 26.5 per cent, and the cop-

per and manganese contents of the alloy being such as to define a point on the accompanying trilinear chart (Fig. 1) lying within an area defined by a line connecting the following series of points:

|    | Point No. | Percent Cu | Percent Mn |
|----|-----------|------------|------------|
| 10 | 10        | 0          | 33.3       |
|    | 11        | 5          | 26         |
|    | 12        | 10         | 18         |
|    | 13        | 15         | 12         |
|    | 24        | 16         | 10         |
|    | 14        | 20         | 7.5        |
|    | 25        | 20         | 10         |
|    | 20        | 20         | 12.7       |
|    | 15        | 25         | 17         |
|    | 16        | 28         | 17.5       |
| 15 | 21        | 28.5       | 20         |
|    | 18        | 26         | 23         |
|    | 19        | 25         | 26         |
|    | 22        | 23.3       | 30         |
|    | 15'       | 25         | 31         |
|    | 14'       | 20         | 36         |
|    | 13'       | 15         | 41         |
|    | 28        | 11         | 44.5       |
|    | 12'       | 10         | 45         |
|    | 23        | 7.5        | 45.7       |
| 20 | 11'       | 5          | 47         |
|    | 10'       | 0          | 48.5       |
|    | 10        | 0          | 33.3       |
|    | 25        |            |            |

EDMUND A. ANDERSON.  
GERALD EDMUND.